

# UNITED STATES PATENT OFFICE.

CARL DITTMAR, OF NEW YORK, N. Y.

## EXPLOSIVE COMPOUND.

SPECIFICATION forming part of Letters Patent No. 252,600, dated January 24, 1882.

Application filed November 7, 1881. (No specimens.)

*To all whom it may concern:*

Be it known that I, CARL DITTMAR, of the city of New York, county of New York, and State of New York, have invented a new and useful Explosive Compound, which I provisionally term "Chlornitrosaccharose," which compound is fully described in the following specification.

This invention relates to the class of high explosive compounds, and is intended to supplant nitro-glycerine and its combination with other materials on account of its cheapness and its greater safety in manufacture, use, and transportation.

Hitherto it has been very difficult to free nitro-sugar from the superfluous acid remaining after nitroing cane-sugar or sucrose. It is best to have the sugar dissolved in some liquid which would also combine with nitric acid in order to nitro the sugar thoroughly and to be able to wash the superfluous acid out afterward. Glycerine has been used to dissolve cane-sugar or sucrose, and the solution was nitroed afterward; but the glycerine does not dissolve sugar very readily, and the temperature rises very high and quick while mixing the acids with the glycerine-sugar. I have tried many other liquids; but I found chlorhydrin best for dissolving cane-sugar or sucrose for subsequently nitroing, as it dissolves more sugar than common glycerine does, and the temperature rises much less than when the chlorhydrin sugar is treated with a mixture of nitric and sulphuric acid than it does with a mixture of sugar and common glycerine.

I manufacture the new compound as follows: I take, for instance, ten parts of chlorhydrin ( $C_3H_7ClO_2$ ) and dissolve in it by gentle heat from three to six parts or more of white sugar. Of this mixture I take one part and mix it in seven parts of a mixture of sulphuric and nitric acid as it is known to be used in the manufacture of gun-cotton, &c. The mixture of chlorhydrin and cane sugar or sucrose can be put in the acid bath quicker than a mixture of glycerine and cane-sugar or sucrose, as the temperature does not rise as high and the compound does not take fire as easily. Therefore the manufacture of chlornitrosaccharose is not so dangerous as the manufacture of nitro-sugar in

combination with glycerine. The compound must be thoroughly washed out from superfluous acid, as any other nitro compound.

The chlornitrosaccharose can be mixed with any other material to make powders of different grades of strength. For instance, from forty to eighty parts of chlornitrosaccharose can be combined with from sixty to twenty parts of similar mixtures as are used in the manufacture of dualin and other explosive compounds of the same character; but if a very large percentage of cane-sugar or sucrose has been used it is too thick to mix it with other materials, and it must be thinned with or dissolved in other liquids—for instance, in wood alcohol, or any other liquid which would combine with or dissolve the chlornitrosaccharose.

The chlornitrosaccharose needs a very strong exploding-cap to explode it, and it is not as liable to explode by concussion as nitro-glycerine is. Therefore any mixture with other materials is not intended to make the compound safer, but to make it cheaper. It is cheaper than nitro-glycerine, as the price of glycerine is more than three times higher than that of sugar.

If the chlornitrosaccharose is combined with other combustible or explosive materials—for instance, fifty parts of chlornitrosaccharose with fifty parts of nitro-cellulose or fifty parts of common black powder or its equivalent—it can be used without an exploding-cap. As the chlornitrosaccharose is not as sensitive to concussion as nitro-glycerine, its combination with other explosive materials can be made very useful for fire-arms.

What I claim as my invention is—

1. The process for forming a new explosive compound, which consists in the formation of a chlornitrosaccharose or nitro-sugar by dissolving cane-sugar or sucrose in chlorhydrin and then converting the same into a nitro compound, substantially as described.

2. The compound hereinbefore described, provisionally termed "chlornitrosaccharose."

CARL DITTMAR.

Witnesses:

WM. H. FORAN,  
JAMES F. THOMSON.